

Patented Jan. 10, 1933

1,893,924

*aqueous sodium silicate and*  
*silicate 90%*  
*trisodium phosphate*

## UNITED STATES PATENT OFFICE

FRANK O. WOODRUFF, OF NEWTON, MASSACHUSETTS, ASSIGNOR TO HARRY H. BECKWITH, OF BROOKLINE, MASSACHUSETTS

## MANUFACTURE OF SHOE STIFFENER MATERIAL

36-68

No Drawing. Application filed August 12, 1931. Serial No. 556,615.

There are various kinds of shoe stiffener materials which go into the manufacture of shoe stiffener parts, such as box toes and counters. One of the important kinds of shoe stiffener material contains distributed therethrough nitrocellulose or celluloid, which renders the material susceptible of being converted into a limp and mouldable condition by the use of various organic solvents. It is the practice, therefore, to treat box toe or counter blanks of such material with a suitable organic solvent to render them limp and mouldable, in which condition they are assembled and moulded with the shoe upper and then permitted to set in place. This conditioning treatment with solvents may be performed either at the factory where the shoe stiffener material is made, or at the shoe factory. When the shoe stiffener blanks are treated before shipping to the shoe factory, they are usually packed in hermetically sealed containers so that they can be maintained in limp and mouldable condition until they are applied to the shoe. A major objection, especially from the point of view of the shoe manufacturer, to shoe stiffener parts containing nitrocellulose or celluloid as the stiffening agent is that they are highly inflammable and give rise to serious fire and explosion hazard, especially when the nitrocellulose is present, as is customarily the case, in a fabric or felt which itself is made of combustible material like cellulose fiber. It must be borne in mind that shoe stiffener material containing nitrocellulose or celluloid is not only dangerous because it is readily set on fire through carelessness, but that it is inherently dangerous on account of the liability of the nitrocellulose to undergo spontaneous decomposition and ignition. I have found that it is possible to stabilize shoe stiffener material consisting of a fabric or felt foundation associated with nitrocellulose or celluloid, by the use of various chemicals of an alkaline nature. The alkaline chemicals which I have found to be most desirable are those which impart to the stiffener material high fire resistance and, at the same time permit the material to be rendered limp and mouldable by the action of the usual nitrocellulose or celluloid solvents. I have found that when shoe stiffener material consisting, for example, of woven cotton fabric coated or impregnated with celluloid, is treated with a concentrated sodium silicate solution and then dried, not only is the stiffener material rendered more stable, but acquires high fire resistance. One of the difficulties presented when sodium silicate alone is used, however, is that the stiffener material containing nitrocellulose does not acquire the desired limpness and mouldability upon treatment with nitrocellulose solvents. Evidently, the sodium silicate not only forms fireproof sheathings on the combustible fiber, but also deposits on the nitrocellulose as continuous films or coatings which are penetrated only slowly, if at all, by the nitrocellulose solvent. I have discovered that the impermeability of the sodium silicate films is destroyed when a crystallizable alkaline salt, preferably one which crystallizes with water of hydration or crystallization, is used as well as the sodium silicate solution. Apparently, salts which crystallize with water of hydration or crystallization break up the continuity of the sodium silicate sheathings or films sufficiently to permit nitrocellulose solvents to come in contact quickly with the nitrocellulose and thus to gelatinize the same practically as quickly as if no sodium silicate were present. It may be that the crystallizable salt breaks up the continuity of the sodium silicate films by abstracting water therefrom and thereby satisfying its own water of crystallization, but this is merely advanced as speculation or theory. While various alkaline salts which crystallize from aqueous solution with water of crystallization may be employed, I prefer to use salts of the character of the water-soluble phosphates and carbonates, first, for the reason that they can be admixed with the sodium silicate solution to form a single solution without any observable reaction, and, second, because they, themselves, are highly combustible and impart this property to the stiffener material. In this connection, it is well to observe that a soluble phosphate, such as

tri-sodium phosphate, crystallizes from aqueous solution with 12 molecules of water of crystallization. Moreover, the phosphate radical, as is well known, is markedly fire-resistant and imparts this property to combustible materials to which it is applied. The soluble carbonates, such as ammonium carbonate and sodium carbonate, are not only valuable because of their water of crystallization, but more especially because they decompose under the action of heat to liberate incombustible gases which inhibit combustion. Thus, ammonium carbonate undergoes decomposition when heated to liberate both carbon dioxide and ammonia, both of which are incombustible and accordingly smother a fire. In point of fact, the soluble carbonates, especially ammonium carbonate, alone may be used to impart high fire resistance to the stiffener material, although I prefer to use them conjunctively with a solution of sodium silicate, because the combination of the two salts is more effective in this respect than the carbonate alone. The soluble phosphates, however, such as tri-sodium phosphate, should be used with the silicate, for the reason that such phosphates alone are not sufficiently effective in lowering the combustibility of stiffening material containing nitrocellulose, even though the foundation alone might be rendered non-combustible by such phosphate alone.

While it is possible to practise various specific procedures falling within the ambit of the present invention, a procedure which has been found to give eminently satisfactory results is carried out about as follows. A single or multi-ply cotton fabric which has been coated or impregnated with a solution of nitrocellulose or celluloid and then dried to form shoe stiffener material, may be submersed in a concentrated solution of both tri-sodium phosphate and sodium silicate. The solution may, for example, be made up by adding 20 parts of sodium silicate of 38° Baumé and 30 parts of tri-sodium phosphate ( $Na_3PO_4 \cdot 12H_2O$ ) to 50 parts of water, preferably with the application of heat so as to promote rapid dissolution. The sodium silicate and tri-sodium phosphate form a homogeneous, colorless and limpid solution. In order to promote penetration of the solution into the fabric, the solution is preferably heated to and kept at about boiling temperature (212° F.), at which temperature a period of immersion of only about 30 seconds is sufficient to associate sufficient salt with the nitrocellulose-containing fabric to impart the desired properties thereto. The solution-soaked fabric may then be drained free of excess solution and dried. The impregnation and drying of the stiffening material may be practised as a continuous process, as the stiffening material may be un-wound from a roll, then passed through a

bath of the solution at a rate to ensure satisfactory impregnation, and finally over a drum dryer. The dried material is incom-  
70 bustible to such an extent that when a flame is applied thereto only smoldering takes place and there is a decided tendency for the smoldering to die out. In fact, when the flame is removed from the material, such little combustion as has been set up tends to cease, and no creeping of the glow to the un-fired portions of the material is observable.  
75

In the absence of my treatment, when the nitrocellulose-containing fabric is set on fire, even though the flame is extinguished, the residual glow continues to creep to the un-fired portions of the fabric with attendant liberation of considerable heat and white, choking fumes of nitrous oxides.  
80

Aside from the incombustibility of the treated material when it is deliberately fired, there is no tendency whatever for it to undergo spontaneous combustion and ignition. In other words, the agents incorporated into the material have a tremendous stabilizing effect thereon, by virtue of the fact that they are alkaline and thus can neutralize nitrous oxide fumes into which the nitrocellulose might tend to decompose with the evolution of heat under certain conditions.  
85

The principles of the present invention extend to various types of foundations into which nitrocellulose or celluloid has been incorporated to form shoe stiffening material. For example, the shoe stiffening material may be one which has been fabricated on a paper machine and throughout which nitrocellulose in fibrous or precipitated form has been incorporated, as by mixing the fibrous or precipitated nitrocellulose with unnitrat-  
100 ed cellulose fiber in the beater engine prior to sheeting. So, too, a foundation fabricated on machinery of the textile or paper-making type may be coated or impregnated with a nitrocellulose or celluloid solution and then dried to produce shoe stiffening material.  
105 Any one of these foundations containing nitrocellulose or celluloid either as a continuous phase, by virtue of treatment with a solution of nitrocellulose or celluloid, or as a discontinuous phase, by virtue of the incorporation thereto of fibrous nitrocellulose or precipitated nitrocellulose, may be subjected to the stabilizing and fireproofing treatment of my invention.  
110

I would not regard it as a departure from the teaching of my invention if one were to impregnate the nitrocellulose-containing foundation first with the sodium silicate solution and then with an aqueous solution of the crystallizable alkaline salt, such as tri-sodium phosphate, with or without intermediate drying, but it is obviously preferable to use the two salts in a single solution and thus to effect impregnation of the founda-  
115  
120  
125  
130

tion in a single step and then to follow such impregnation by drying.

In the appended claims, I am using the term "nitrocellulose" as meaning either nitrocellulose as such or nitrocellulose which has been compounded with other materials, such as camphor, to produce celluloid or analogous nitrocellulose compounds.

I claim:

- 10 1. Fire-resistant shoe stiffener material comprising a fibrous foundation associated with nitrocellulose as a stiffening agent and impregnated with a mixture of both sodium silicate and a crystallized alkaline salt, said material being rendered limp and mouldable by treatment with a nitrocellulose solvent.
- 15 2. Fire-resistant shoe stiffener material comprising a fibrous foundation associated with nitrocellulose as a stiffening agent and impregnated with a mixture of both sodium silicate and a hydrated, crystallized alkaline salt, said material being rendered limp and mouldable by treatment with a nitrocellulose solvent.
- 20 3. Fire-resistant shoe stiffener material comprising a fibrous foundation associated with nitrocellulose as a stiffening agent and impregnated with a mixture of both sodium silicate and a crystallized water-soluble phosphate, said material being rendered limp and mouldable by treatment with a nitrocellulose solvent.
- 25 4. Fire-resistant shoe stiffener material comprising a fibrous foundation associated with nitrocellulose as a stiffening agent and impregnated with a mixture of both sodium silicate and crystallized tri-sodium phosphate, said material being rendered limp and mouldable by treatment with a nitrocellulose solvent.
- 30 5. Fire-resistant shoe stiffener material comprising a fibrous foundation associated with nitrocellulose as a stiffening agent and impregnated with a mixture of both sodium silicate and a crystallized water-soluble carbonate, said material being rendered limp and mouldable by treatment with a nitrocellulose solvent.
- 35 6. Fire-resistant shoe stiffener material comprising a fibrous foundation associated with nitrocellulose as a stiffening agent and impregnated with a mixture of both sodium silicate and crystallized ammonium carbonate, said material being rendered limp and mouldable by treatment with a nitrocellulose solvent.
- 40 7. A process which comprises impregnating a fibrous foundation containing nitrocellulose with an aqueous solution of both sodium silicate and a crystallizable alkaline salt of the character of the soluble phosphates and carbonates, and drying the impregnated foundation.
- 45 8. A process which comprises impregnating a fibrous foundation containing nitro-

cellulose with a concentrated solution of both sodium silicate and tri-sodium phosphate, and drying the impregnated foundation.

9. A process which comprises impregnating a fibrous foundation containing nitrocellulose with a concentrated solution of both sodium silicate and tri-sodium phosphate, drying the impregnated foundation, and cutting the dried foundation into shoe stiffener parts.

10. A process which comprises impregnating a fibrous foundation containing nitrocellulose with an aqueous solution made up of about 50 parts of water, 20 parts of sodium silicate of 38° Baumé, and 30 parts of tri-sodium phosphate (Na<sub>3</sub>PO<sub>4</sub>·H<sub>2</sub>O), drying the impregnated foundation, and cutting the dried foundation into shoe stiffener parts.

In testimony whereof I have affixed my signature.

FRANK O. WOODRUFF.

75

80

85

90

95

100

105

110

115

120

125

130